

# UNITED STATES PATENT OFFICE.

ALBERT C. HOLZAPFEL, OF NEW YORK, N. Y.

## SURFACE-COATING COMPOSITION.

1,379,018.

Specification of Letters Patent. Patented May 24, 1921.

No Drawing.

Application filed May 25, 1920. Serial No. 384,174.

To all whom it may concern:

Be it known that I, ALBERT C. HOLZAPFEL, a subject of the King of Great Britain, residing at New York, in the county of New York and State of New York, have invented certain new and useful Improvements in Surface-Coating Compositions, of which the following is a specification.

This invention relates to a surface coating composition such as a paint, varnish, or the like, primarily intended for coating metal, and particularly iron and steel, but adapted for coating wood and other materials.

15 Pitches derived from the treatment of oils and fats, such as stearin pitch, palm oil pitch, and the like, have been used in the manufacture of surface coating compositions, as for example, the surface coating

20 composition described in Letters Patent No. 1,313,252, granted to Paul Walther and me May 4, 1920. In such compositions, gums such as copal, dammar and the like have been used, and it has heretofore been consid-

25 ered essential to employ such gums in producing a paint, varnish, or the like, in which pitch derived from the treatment of oils and fats is present as a material or substantial ingredient.

30 Now, I have discovered that a satisfactory varnish or vehicle for the pigment if the composition is used in the manufacture of paint, can be made from pitch derived from the treatment of oils and fats by

35 merely dissolving from approximately 30 to 40 parts of it by weight in from 60 to 70 parts by weight of tar oil such as a distillate of tar oil, of from 70° to 120° flash-point, or other hydrocarbon solvent of the 40 pitch, without the employment of copal, dammar, or other gum heretofore used therewith.

If the composition is to be used in the manufacture of paint, from approximately 45 1 to 50 and preferably from 20 to 50 parts by weight of a suitable pigment is incorporated therein.

Linseed oil or any of the oils commonly used in the manufacture of oil paints may 50 be added to the composition either with or without the pigment, but the addition of such oil is not necessary. If such oil is used, I prefer to add it in approximately the proportions of from approximately 5 to 55 20 parts by weight to from 80 to 95 parts by weight of the solution of the stearin or

other pitch derived from the treatment of oils or fats.

The preferred proportions of the pitch to the solvent will vary chiefly according to 60 the character of the pitch used, the season of the year and the temperature at which the varnish or paint is to be applied, as will be readily understood by those skilled in the art. It is to be understood that these proportions may vary widely within the limits of the solubility of the pitch in the solvent used, but the proportions set forth above have been found to be most satisfactory. Similarly, the proportions of the linseed or 70 other similar oil to the pitch solution may vary within wide limits, but the oil should not be added in excess of 20 per cent. by weight of the whole.

It is to be understood that while tar oil 75 such as a distillate of tar oil of from 70° to 120° flashpoint—is preferred as the solvent for the stearin or like pitch, other hydrocarbon solvents may be used with a considerable measure of success and are, to 80 such extent, equivalents of the tar oil. Similarly, while I prefer to employ linseed oil, if a paint oil is employed, other paint oils are to be regarded as equivalents of the linseed oil for use in my composition. 85

The varnish or the paint produced in accordance with my invention is applied in the usual way, either by brush or spray, and dries rapidly, usually within an hour, with a good, smooth gloss. 90

I claim:

1. A surface coating composition consisting of approximately from 30 to 40 parts by weight of pitch derived from the treatment of oils and fats and from 60 to 70 95 parts by weight of a hydrocarbon solvent.

2. A surface coating composition consisting of approximately from 30 to 40 parts by weight of pitch derived from the treatment of oils and fats and from 60 to 70 100 parts by weight of tar oil.

3. A surface coating composition consisting of approximately from 30 to 40 parts by weight of stearin pitch and from 60 to 70 parts by weight of tar oil. 105

4. A surface coating composition consisting of approximately from 30 to 40 parts by weight of pitch derived from the treatment of fats and oils, from 60 to 70 parts by weight of tar oil, and approximately 110 from 1 to 50 parts by weight of pigment.

5. A surface coating composition consist-

ing of approximately from 30 to 40 parts by weight of stearin pitch, from 60 to 70 parts by weight of tar oil, and approximately from 1 to 50 parts by weight of 5 pigment.

6. A surface coating composition consisting of approximately from 30 to 40 parts by weight of stearin pitch, from 60 to 70 parts by weight of tar oil, and approximately 10 from 20 to 50 parts by weight of pigment.

7. A surface coating composition consisting of approximately from 30 to 40 parts by weight of pitch derived from the treatment 15 of oils and fats, from 60 to 70 parts by weight of tar oil, a pigment, and a paint oil.

8. A surface coating composition consisting of approximately from 30 to 40 parts by weight of pitch derived from the treatment 20

ment of oils and fats, from 60 to 70 parts by weight of tar oil, approximately from 20 to 50 parts by weight of pigment, and not to exceed 20 parts by weight of a paint oil.

9. A surface coating composition consisting of approximately from 30 to 40 parts by weight of stearin pitch, from 60 to 70 parts by weight of tar oil, approximately 25 from 20 to 50 parts by weight of a pigment, and not to exceed 20 parts by weight of linseed oil.

In testimony whereof I affix my signature, in presence of two witnesses.

ALBERT C. HOLZAPFEL

Witnesses:

HELEN A. McCANN,  
H. E. TEHAN.